

**1**

2,900,322

**LUBRICATING OIL CONTAINING A WAX POUR POINT AND CLOUD POINT SUPPRESSER**

Herman J. Zoeller, Union, N.J., assignor to Esso Research and Engineering Company, a corporation of Delaware

No Drawing. Application August 6, 1956  
Serial No. 602,441

4 Claims. (Cl. 208—19)

The present invention relates to improvements in the cloud and haze properties of lubricating oils, diesel oils, transformer oils, and similar petroleum oils which are often used or stored at low temperatures. More particularly, the present invention relates to the reduction of the haze and cloud points of these oils by a new and improved incorporation of an inhibitor therein.

The unsatisfactory performance of lubricating oils and diesel fuels at cold temperatures and in cold climates is a problem that has been with the petroleum industry a long time. The problem has been traced to small amounts of wax in the oils. Below a critical temperature, the cloud point of the oil, the wax begins to solidify. If the oil is a diesel fuel, the solids thus formed may block filters in the fuel system and eventually cause fuel starvation of the engine. In the case of lubricating oils, the precipitated wax increases the viscosity of the oil and makes proper lubrication difficult.

Conventional dewaxing operations, solvent dewaxing processes for example, are not always feasible nor satisfactory. These are expensive processing steps and their costs often cannot be justified. Many refineries produce lubricating oils from crudes having low wax contents, such as naphthenic crudes. The amount of wax in such oils is not enough to warrant a conventional dewaxing treatment, which necessitates the use of expensive solvents, compressors, refrigerants, filtration equipment and the like. Yet the small amount of wax present, of the order of up to 3%, at +25° F. pour point is enough to disqualify the lubes as low cold test oils. The same is true for diesel fuels.

Other processing steps, such as clay treating, acid treating, and phenol extraction do not have a significant effect on the haze point.

As little as 0.1 to 0.5% of suspended wax crystals in low cold test lubes causes haze, and only 0.15% of wax will raise the haze point 30° F.

Hydrocarbon oils which contain waxy constituents thus often lose their limpidity due to the separation of these solid wax particles, which appear either in the form of a cloud within the oil or as a more or less crystalline precipitate which may remain dispersed throughout the oil. Frequently the separated wax collects on the walls of the container, particularly near the surface of the oil. Such separation often occurs at temperatures which are substantially above the congealing temperature, or pour point of the oil, with the result that small constrictions in a

**2**

lubricating or fuel system may become obstructed. This separation of solid wax is manifested both in the formation of clouds of dispersed precipitate and in the formation of surface wax.

- 5 It is an object of the present invention to provide a process for reducing or preventing the separation of such particles of wax by the addition to the oil of an additive that does not itself contribute to the formation of wax and cloud.
- 10 Other objects and advantages of the present invention will be readily apparent from the more detailed description of the invention hereinafter.

It has now been found that excellent cloud and haze reduction in wax-containing oils may be obtained by adding to these oils small amounts of narrow-boiling, low-melting point hydrocarbon mixtures of a definite composition. More specifically, this reduction is obtained by adding small amounts, .001 to .02% by weight, of paraffin wax melting in the range of about 100° to 118° F. which consists of a substantial proportion of non-normal paraffin waxes. Still more specifically, paraffin wax compositions melting in the range of 100° to 118° F. and composed of from about 45% to 55% normal paraffins in the C<sub>20</sub>—C<sub>30</sub> molecular weight range, 20% to 25% isoparaffins, and about 20% to 25% naphthenes are especially effective in reducing cloud points of lubricating oils, even when added in amounts as low as from 0.001 to 0.005% by weight.

It is customary to add certain compositions to lubricating oils to lower the congealing, or pour point of the oil. 30 These additives, such as the condensation products of aromatics and long chain alkyl halides, generally have no effect upon the cloud or haze point of an oil, and sometimes even raise the latter. The inhibitor composition of the present invention, however, has no particular effect 35 upon the pour point of the oil, but has a marked effect in preventing or retarding the separation of finely divided wax particles. The cloud point inhibitor of the present invention, therefore, may be employed in compositions with conventional pour depressants.

40 The cloud inhibitor may be added to the oils at elevated temperatures. It is often desirable to dissolve a large amount of the inhibitor in a small quantity of oil and then to add this concentrate to the main body of oil at ordinary temperatures. In general, because of the high effectiveness of the inhibitor, about .001 to .005% by weight is employed. Higher concentrations tend to increase the pour point and may increase the cloud and haze as well.

45 The cloud and haze inhibitor compositions of the present invention may readily be prepared from commercial refined paraffin wax containing at least 14 to 16 weight percent non-normal paraffins by removing most of the high melting point, high molecular weight normal paraffins with urea or thiourea. There is a critical composition range, however, which limits the amount of n-paraffins which are removed. Thus, effective compositions contain 50 45% to 55% n-paraffins, 15% to 25% isoparaffins, and 15% to 25% naphthenes. A particularly good composition contains these constituents in the ratio of approximately 2-1-1. Other compositions non-reactive to

urea and containing less n-paraffins, and more isoparaffins and naphthenes, have been found not to be effective as cloud point depressants. Similarly, compositions having a greater proportion of normal paraffins tend to raise the pour point.

To illustrate the effectiveness of the haze and cloud inhibitors of the present invention, the following examples are offered.

In Table I below, there is shown the inspection and composition of the inhibitors of the present invention. For comparative purposes, the effects of four mixtures are shown, designated respectfully by "A," "B," "C" and "D." In column "A" there is shown a commercial grade paraffin wax prepared by solvent de-oiling of a lubricating oil distillate. The source of wax is such that there is at least 14 to 16 weight percent of non-normals therein. The total wax "A" was vacuum distilled to 10% bottoms to concentrate the non-normals. Then the bottoms were treated with urea to separate the high melting point, high molecular weight normal paraffins. The non-reactive material is labeled "Inhibitor B."

A separate portion of the total wax "A" was solvent re-crystallized at +65° F. to remove the high melting normal paraffins as a wax cake, while the filtrate contains most of the low melting point normal and non-normal paraffins. The filtrate wax, after stripping to remove solvent, was urea adducted to separate normal from non-normal paraffins. The non-reactive material is designated "Inhibitor C."

The total wax "A" was urea adducted directly with no intermediate processing sequence to separate the high melting, high molecular weight paraffins. The non-reactive material is designated "Inhibitor D."

In all of the urea treats above, similar conditions of treat, temperature, proportions, and the like obtained. Each inhibitor is the urea-non-reactive material except "A," which is the original wax base stock. The lube base stock itself is an extracted low cold test lube oil from coastal-naphthenic type crude. The urea adduction experiments for removal of highly paraffinic components employed 300 weight percent treats at 160° to 165° F. in solvent solution with 5% water as promoter.

TABLE I

## Cloud point reduction of lube oil

## PART A.—PREPARATION AND INSPECTION OF INHIBITORS

|                                                | A       | B       | C       | D       |
|------------------------------------------------|---------|---------|---------|---------|
| Yield, Wt. percent on "A"-----                 | 100     | 4.1     | 19      | 27      |
| Melting point, ° F.-----                       | 130     | 118     | 105     | 115     |
| Percent oil, ASTM-----                         | 0.4     |         |         |         |
| R.I. @ 90° C. (194° F.)-----                   | 1.4244  | 1.4350  | 1.4286  | 1.4269  |
| Boiling Range 5-95% @ 760 mm., ° F.-----       | 750-870 | 850-890 | 770-850 | 760-850 |
| Mass spectrometric analysis<br>(Mol. percent): |         |         |         |         |
| n-Paraffin-----                                | 87      | 11      | 49      | 54      |
| Isoparaffin-----                               | 9       | 43      | 25      | 26      |
| Naphthene-----                                 | 4       | 38      | 24      | 19      |
| Cond. Naphthene-----                           | 0       | 5       | 0       | 0       |
| Mono-Aromatic-----                             | 0       | 3       | 2       | 1       |

## PART B.—EFFECTIVENESS OF INHIBITORS AS CLOUD POINT DEPRESSANTS

| 5  | Inhibitor | Weight percent | ASTM Pour, ° F. | ASTM Cloud, ° F. |
|----|-----------|----------------|-----------------|------------------|
| 10 | None----- | None           | +20             | +48              |
|    | "A"-----  | 0.001          | +20             | +32              |
|    | "A"-----  | 0.005          | +20             | +36              |
|    | "A"-----  | 0.2            | +30             | +54              |
|    | "B"-----  | 0.001          | +10             | +32              |
|    | "B"-----  | 0.005          | +20             | +32              |
|    | "B"-----  | 0.2            | +25             | +50              |
|    | "C"-----  | 0.001          | +15             | +20              |
|    | "C"-----  | 0.005          | +15             | +22              |
|    | "C"-----  | 0.2            | +25             | +48              |
|    | "D"-----  | 0.001          | +20             | +22              |
|    | "D"-----  | 0.005          | +20             | +22              |
| 15 | "D"-----  | 0.2            | +25             | +52              |

The superiority of the composition of the present invention as a cloud point inhibitor is clearly shown when compared with cloud point inhibitors suggested by the art. One such inhibitor is montan wax. The latter requires an initial bleaching operation to make it suitable for incorporation into wax compositions. In Table II below, is shown the effect of adding small amounts of montan wax to a raffinate obtained by extracting low cold test lubricating oil from a Tia Juana naphthenic type crude. It will be noted that, in the concentrations in which the additive of the invention is effective, substantially no cloud point reduction was realized with the montan wax.

30

TABLE II

| 30 | Inhibitor                | Weight percent   | ASTM Pour, ° F. | ASTM Cloud, ° F. |
|----|--------------------------|------------------|-----------------|------------------|
| 35 | None-----                | None             | +20             | +46              |
|    | Bleached Montan Wax----- | { 0.001<br>0.005 | +15<br>+20      | +50<br>+46       |

What is claimed is:

1. A hydrocarbon oil to which has been added as a haze and cloud point suppressor from about 0.001% to about 0.02% by weight of a petroleum wax composition melting in the range between about 100° F. and about 118° F., said composition containing about 45 to 55 mol. percent of normal paraffin waxes, about 15 to 25 mol. percent of isoparaffin waxes, and about 15 to 25 mol. percent of naphthenic waxes.

2. An oil as defined by claim 1 wherein said wax composition contains normal paraffin, isoparaffin and naphthenic waxes in a mol. ratio of about 2/1/1.

3. An oil as defined by claim 1 wherein said wax composition is present in a concentration of from about 0.001% to about 0.005% by weight.

4. An oil as defined by claim 1 wherein said wax composition is employed in conjunction with a pour point depressant.

References Cited in the file of this patent

UNITED STATES PATENTS

60 2,671,051 Moore ----- Mar. 2, 1954